

May 31, 1966

S. ILNYCKYJ

3,254,063

## PROCESS FOR PREPARATION OF POUR DEPRESSANTS

Filed Jan. 4, 1962



Stephan Ilnyckyj

## Inventor

By W. O. Kilman

## Patent Attorney

1

3,254,063

**PROCESS FOR PREPARATION OF  
POUR DEPRESSANTS**

Stephen Ilnyckyj, Sarnia, Ontario, Canada, assignor to  
Esso Research and Engineering Company, a corporation  
of Delaware

Filed Jan. 4, 1962, Ser. No. 164,248  
11 Claims. (Cl. 260—87.3)

The present invention is concerned with the manufacture of improved pour depressants, particularly for use with middle distillates. The pour depressant of the present invention comprises copolymers of ethylene with up to about 50% by weight of an olefinically unsaturated aliphatic monomer containing from about 3 to 5 carbon atoms per molecule. The copolymers of a particular average molecular weight are obtained by controlling the conditions of reaction. The preferred copolymer of the present invention is a particular copolymer of ethylene and vinyl acetate.

The present application is a continuation-in-part of Ser. No. 1,838 filed Jan. 5, 1960, U.S. Patent No. 3,093,623 entitled Process for the Manufacture of Improved Pour Depressants for Middle Distillates, Inventor Stephan Ilnyckyj, which in turn is a continuation-in-part of Ser. No. 835,587 filed Aug. 24, 1959, now abandoned entitled Process for the Manufacture of Improved Pour Depressants for Middle Distillates, Inventor, Stephan Ilnyckyj.

In accordance with the present invention, pour depressants of improved potency are secured by utilizing relatively small quantities of mercaptans or carbon tetrachloride during the copolymerization step.

With the increase in the use of hydrocarbon fuels of all kinds, a serious problem has arisen in areas frequently subjected to low temperatures in the cold test characteristics of fuels. Particularly, serious problems have been encountered with heating oils and diesel and jet fuels that have too high a pour point, resulting either in distributional or operating difficulties or both. For example, the distribution of heating oils by pumping or syphoning is rendered difficult or impossible at temperatures around or below the pour point of the oil. Furthermore, the flow of the oil at such temperatures through the filters cannot be maintained, leading to the failure of the equipment to operate.

Also the low temperature properties of petroleum distillate fuels boiling in the range between about 250° and about 750° F. have attracted increasing attention in recent years because of the growth of market for such fuels in subarctic areas and because of the development of turbo-jet aircraft capable of operating at altitudes where temperatures of —50° F. or lower may be encountered.

It is, therefore, an object of the present invention to set forth an improved process for the manufacture of very effective pour depressants for middle distillates and lighter oils. In general, these oils boil in the range from about 250° to 750° F.

It is a still further object of the present invention to provide heating oils, diesel fuel oils, kerosenes and jet fuels having low pour points. Aviation turbo-jet fuels in which the polymers may be used normally boil between about 250° and about 550° F. and are used in both military and civilian aircraft. Such fuels are more fully defined by U.S. military specifications MIL-F-5624C, MIL-F-25554A, MIL-F-25558A, and amendments thereto. Kerosenes and heating oils will normally have boiling ranges between about 300° and about 750° F. and are more fully described in ASTM specification D-396-48T and supplements thereto, where they are referred to as No. 1 and No. 2 fuel oils. Diesel fuels in which the polymers may be employed are described in detail in ASTM specification D-975-53T and later versions of the same specification.

2

The process of the present invention produces copolymers of ethylene and up to about 50% by weight of an olefinically unsaturated aliphatic monomer containing from about 3 to 5 carbon atoms per molecule. In general, these compounds may comprise vinyl acetate, vinyl propionate, methyl methacrylate, allyl ethyl ether, divinyl ether, acrylonitrile, vinylacetonitrile and the like.

The preferred copolymers comprise ethylene-vinyl acetate copolymer. It is preferred that the parts by weight of ethylene in the copolymer be in the range from about 60 to 99% as compared to parts by weight of vinyl acetate in the range from about 40 to about 1%. A very desirable polyethylene vinyl acetate copolymer contains about 15% to 28% by weight of vinyl acetate as, for example, about 20 parts by weight of vinyl acetate.

The molecular weights of the ethylene-vinyl acetate copolymer are critical and should be in the range from about 1,000 to 3,000, preferably in the range from about 1,500 to 2,200. The molecular weights are determined by K. Rast's method (Ber. 55, 1051, 3727 (1922)).

The ethylene-vinyl acetate copolymer as described above is used in a concentration in the range from about .001 to 0.2% by weight, preferably in a concentration in the range from about .005 to 0.1% by weight.

In accordance with the present invention, the polymerization process is conducted in a solvent as, for example, toluene or hexane. It is preferred, however, to use a benzene solvent. The initiator comprises any peroxy compound, preferably di-tertiary-butyl-peroxide. The temperature of the polymerization reaction is in the range from about 280° to 340° F. A very desirable temperature is about 300° F. The pressure is in the range from about 700 to 2,000 pounds, preferably 800 or 900 pounds. The autoclave or similar equipment containing the solvent, initiator and vinyl acetate is purged with nitrogen, then with ethylene before charging with a sufficient amount of ethylene to yield the desired pressure when heated to the reaction temperature. During the polymerization, additional ethylene is added to maintain the pressure at the desired level. Polymerization is considered complete when the pressure drops less than 50 p.s.i.g. per hour. The product is stripped free of solvent and unreacted vinyl acetate under vacuum.

The present invention may be more fully understood by reference to the drawing illustrating one embodiment of the same. Referring specifically to the drawing, reactor 1 is first purged with nitrogen, introduced by means of line 2 and pump 3. Reactor 1 is then purged with ethylene which is introduced by means of line 2 and pump 3. Gases are removed from reactor 1 by means of line 4. The reactor is maintained at a positive pressure in the range from about 50 to 100 pounds absolute.

Approximately 220 parts by weight of benzene is introduced into reactor 1 from benzene storage 5 by means of line 6 and pump 7. Reactor 1 is then raised to a temperature of 300° F. by means of heating element 8 wherein a heating fluid or equivalent is introduced by means of line 9 and withdrawn by means of line 10. Reactor 1 is held at 300° F. during the course of the reaction by the removal of heat or by the addition of heat thereto. Ethylene is introduced by means of line 2 so as to raise the pressure of the reactor to about 900 pounds.

The addition of vinyl acetate and of di-tertiary-butyl-peroxide is started concurrently. The vinyl acetate is withdrawn from storage zone 11 and introduced into the reactor by means of line 12 and pump 13. Approximately 55 parts by weight of vinyl acetate is added over a two hour period. The peroxide is introduced by passing benzene into storage zone 14 by means of line 15 and then introducing the solution into the reactor 1 by means of line 16 and pump 17. Approximately 5.5 parts by weight of peroxide are combined with 16.5 parts by

weight of benzene. The resulting 22 parts by weight of 25% peroxide solution in benzene is added to reactor 1 over a three hour period.

In accordance with the present invention, during the addition of the vinyl acetate a mercaptan as, for example, dodecyl mercaptan is continuously added by means of line 18. The amount of mercaptan added to the reaction mixture is such as to yield .02 to .4 wt. percent, preferably .1 to .2 wt. percent of mercaptan sulfur per total amount of vinyl acetate used in the copolymerization.

After the addition of the peroxide has been completed, the reactor is held for an additional one-half hour at a temperature of about 300° F. The ethylene is added continuously so as to maintain the pressure at about 900 pounds. In operation, approximately 934 parts by weight by vinyl acetate are used in conjunction with from about 2,800 to 3,800 parts by weight of ethylene.

At the end of the reaction, the reactor is allowed to cool to about 160° F. and the reaction product is withdrawn by means of line 19 and passed into separation zone 20. Excess ethylene is removed overhead from separation zone 20 by means of line 21. The polymer product comprising the copolymer in a benzene solution may be withdrawn by means of line 22 and further handled as desired. Under certain instances, it may be desirable to separate at least a portion of the benzene from the copolymer. Under these conditions, the benzene copolymer product is passed to separation zone 23 by means of line 24. Benzene is removed overhead by means of line 25, while a copolymer product is withdrawn by means of line 26.

The quantity mentioned above may be somewhat varied. For example, based upon 55 parts by weight of vinyl acetate, the amount of benzene utilized may vary from about 180 to 300 parts by weight, and the amount of di-tertiary-butyl-peroxide may vary from about 3 to 8 parts by weight. Also as mentioned, the amount of ethylene utilized varies from about 2,800 to 3,800 parts by weight, or approximately 938 parts by weight of vinyl acetate. The time of reaction also may be varied from about 2 to 4 hours, depending upon other operating variables.

In order to further illustrate the invention, a number of operations were conducted in accordance with the above described technique. The results of these operations are illustrated in the following table:

*Effect of dodecyl mercaptan and carbon tetrachloride on quality of the pour depressant*

[Conditions of copolymerization: 1800 ml. of benzene, 300 ml. of vinyl acetate over 3 hours, 30 ml. of Di-t-butyl peroxide over 3½ hours, 900 p.s.i.g., 300° F., total reaction time 3½ hours]

| Modifier                                | None  | Dodecyl Mercaptan |       |       |       | Carbon Tetrachloride |       |       |
|-----------------------------------------|-------|-------------------|-------|-------|-------|----------------------|-------|-------|
|                                         |       | 0.33              | 1.0   | 2.0   | 4.0   | 0.33                 | 1.0   | 2.0   |
| Modifier in Vinyl Acetate, vol. percent | Nil   | 0.33              | 1.0   | 2.0   | 4.0   | 0.33                 | 1.0   | 2.0   |
| Yield, g.                               | 797   | 750               | 738   | 679   | 541   | 715                  | 699   | 662   |
| Vinyl Acetate, wt. percent              | 23.6  | 29.0              | 27.0  | 30.6  | 30.7  | 34.0                 | 24.6  | 27.1  |
| Molecular Weight                        | 2,700 | 2,700             | 2,950 | 2,685 | 1,750 | 2,440                | 2,475 | 1,800 |
| Viscosity at 100° F., <sup>1</sup> cs.  | 192   | 188               | 150   | 130   | 116   | 161                  | 180   | 161   |
| Pour Depression, <sup>2</sup> ° F.:     |       |                   |       |       |       |                      |       |       |
| With 0.015 wt. percent                  | 30    | 55                | 65    | 65    | 15    | 45                   | 45    | 25    |
| With 0.025 wt. percent                  | 50    | 85                | 85    | 85    | 25    | 70                   | 70    | 45    |

<sup>1</sup> 50/50 solution of copolymer in 400-500° F. naphtha.

<sup>2</sup> In a 50/50 blend of virgin and cracked gas oils, ASTM pour + 20° F.

Thus, it is evident from the above that pour depressants of marked increased potency are secured when utilizing modifiers as, for example, dodecyl mercaptan and carbon tetrachloride during the manufacturing operation.

The mercaptan is preferably an aliphatic mercaptan having 1 to 18 carbon atoms in the molecule, preferably one having from 10 to 14 carbon atoms in the molecule. The amount of mercaptan added to the reaction mixture is preferably added during the addition of the vinyl acetate in an amount such as to yield 0.02 to 0.4 wt. percent, preferably 0.1 to 0.2 wt. percent of mercaptan sulfur

per total amount of vinyl acetate used in the copolymerization. Thus, when utilizing dodecyl mercaptan, the amount used is a concentration equal to 0.1 to 2.0 wt. percent, preferably 0.5 to 1.0 wt. percent of the total amount of vinyl acetate used in the copolymerization.

In accordance with the present invention, the reactants are preferably added continuously to the reactor, as described above.

What is claimed is:

1. Process for the manufacture of a pour depressant comprising a copolymer of ethylene and an aliphatic vinyl monomer which comprises reacting ethylene and said monomer in a benzene solvent at a temperature in the range of from about 280° to 340° F. and at a pressure in the range from about 700 to 2,000 pounds under conditions wherein the concentration of the vinyl monomer in the solvent solution varies from about 4 to 14%, whereby a polymer having a molecular weight in the range from about 1,000 to 3,000 is secured and wherein the concentration of the vinyl acetate in the product will vary from about 1 to 40% and adding to said benzene solvent an aliphatic mercaptan containing from about 1 to 18 carbon atoms in the molecule in a concentration to yield .02 to .4 wt. percent of mercaptan sulfur per total amount of vinyl acetate used in the copolymerization.

2. Process as defined by claim 1 wherein the concentration of the vinyl monomer in the solvent solution varies from about 4 to 7½%, whereby the concentration of the vinyl monomer in the product will vary from about 15 to about 25%.

3. Process for the manufacture of a pour depressant comprising a copolymer of ethylene and an aliphatic vinyl monomer which comprises reacting ethylene and said monomer in a benzene solvent at a temperature in the range of from about 280° to 340° F. and at a pressure in the range from about 700 to 2,000 pounds under conditions wherein the concentration of the vinyl monomer in the solvent solution varies from about 4 to 14%, whereby a polymer having a molecular weight in the range from about 1,000 to 3,000 is secured and wherein the concentration of the vinyl acetate in the product will vary from about 1 to 40% and adding to said benzene solvent a modifier selected from the group consisting of carbon tetrachloride and an aliphatic mercaptan containing from about 1 to 18 carbon atoms in the molecule, said modifier being present in a concentration of from about 0.33 to 1.0% by volume based upon the vinyl acetate.

4. Process as defined by claim 1 wherein said mercaptan contains from about 10 to 14 carbon atoms in the molecule.

5. Process as defined by claim 1 wherein the time period is in the range from about 2 to 6 hours, wherein the temperature is in the range of from about 290° to 310° F., wherein the pressure is in the range from about 650 to 1,000 pounds, and wherein the concentration of the vinyl acetate in a benzene solution varies from about .53 to about 10%.

6. Process as defined by claim 1 wherein the reaction is initiated by a peroxy compound, di-tertiary-butyl-peroxide.

7. Process as defined by claim 1 wherein the reaction is carried out in an autoclave which is purged with nitrogen, then with ethylene and then charged with a sufficient amount of ethylene to yield the desired pressure when heated to the reaction temperature.

8. Process as defined by claim 1 wherein additional ethylene is added to the reaction mixture whenever the pressure drops by about 100 p.s.i.g.

9. Process as defined by claim 1 wherein unreacted vinyl acetate is stripped under vacuum when the reaction is completed.

10. Process as defined by claim 1 wherein said aliphatic mercaptan is dodecyl mercaptan.

11. Process as defined by claim 3 wherein the modifier consists essentially of carbon tetrachloride present in a concentration of about .33-1.0% by volume based upon the volume of vinyl acetate present.

#### References Cited by the Examiner

##### UNITED STATES PATENTS

|   |           |        |         |          |
|---|-----------|--------|---------|----------|
| 5 | 2,395,381 | 2/1946 | Squires | 260-87.3 |
|   | 2,396,785 | 3/1946 | Hanford | 260-87.3 |
|   | 2,947,735 | 8/1960 | Bartl   | 260-87.3 |
|   | 3,093,623 | 6/1963 | Ilnyckj | 260-87.3 |

##### OTHER REFERENCES

Wiles et al.: Industrial and Engineering Chemistry, vol. 10 41, No. 8, pp. 1679-1682.

Schildknecht: Vinyl and Related Polymers, pp. 106 and 504, Wiley (1957).

JOSEPH L. SCHOFER, *Primary Examiner.*

15 LOUISE P. QUAST, JOSEPH R. LIBERMAN, WILLIAM H. SHORT, *Examiners.*

JOHN F. McNALLY, *Assistant Examiner.*